

Oct. 22, 1968

R. H. KROCK ET AL

3,407,048

MOLYBDENUM COMPOSITE MATERIALS AND METHOD OF MAKING THE SAME

Filed Jan. 22, 1968



FIG. 1



FIG. 2

INVENTORS  
EDWARD J. ZDANUK  
RICHARD H. KROCK

*Charles W. Hoffmann*  
ATTORNEY

1

3,407,048

## MOLYBDENUM COMPOSITE MATERIALS AND METHOD OF MAKING THE SAME

Richard H. Krock, Peabody, and Edward J. Zdanuk, Lexington, Mass., assignors to P. R. Mallory & Co. Inc., Indianapolis, Ind., a corporation of Delaware

Filed Jan. 22, 1968, Ser. No. 699,658

8 Claims. (Cl. 29—182.1)

### ABSTRACT OF THE DISCLOSURE

A composite material in which the primary by volume constituent is molybdenum having a low gas content for use as a current carrying material. The composite material consists essentially of a substantially continuous skeleton of integrally bonded molybdenum particles, the voids of which are filled by a substantially continuous matrix of a metal alloy which is substantially mutually insoluble and substantially nonreactive with molybdenum. The alloy matrix includes at least one highly conductive metal and another metal which is less conductive wherein the less conductive metal tends to concentrate at the interface between the molybdenum and the alloy matrix.

The present invention relates to powder metallurgy and, more particularly, to improved means and methods of providing composite materials having a low gas content and low content of materials which may release gas for use as contact materials in current interrupter devices such as switching devices and the like which may operate in a vacuum atmosphere.

Molybdenum is used in electrical contact materials because of its inherent characteristics of hardness and resistance to arcing. Due to the inherent characteristics of molybdenum, molybdenum contacts are less likely to pit than contacts fabricated from copper, silver or gold. However, pure molybdenum contacts possess high electrical resistance which lowers the efficiency and reliability of the molybdenum contact materials. Pure copper, silver, or gold contact materials have good thermal and conductivity characteristics but are likely to experience arc erosion and contact welding.

It is thought that a contact material composed essentially of a continuous skeleton of bonded molybdenum particles integrally joined with a continuous matrix material which has good thermal and electrical properties and which is substantially mutually insoluble and substantially nonreactive with molybdenum might make advantageous use of the several outstanding characteristics of the constituents. For example, if the contact material is composed of a matrix material selected from the group consisting of copper, silver and gold which is alloyed with a reactive metal selected from the group consisting of titanium and zirconium, the alloy being substantially mutually insoluble and substantially nonreactive with molybdenum, it is thought that the composite material will have good current carrying and thermal conductivity properties, hardness, resistance to arc erosion and superior anti-weld properties.

Composites of molybdenum and copper may be prepared by pressing the mixed metal powders into a required shape and subsequently sintering the compacted powders in a hydrogen atmosphere above the melting point temperature of copper, preferably between 1250° and 1350° C. The hydrogen atmosphere appears to act as a flux and the molten copper wets the molybdenum particles and cements the particles together. The copper infiltrant imparts strength and ductility to the molybdenum powder body and also provides the resultant body with higher current carrying capability and thermal conductivity. However, it is noted that the above process

2

makes no attempt to reduce the gas content or content of materials that may release gas during the operation of the material in switching devices operating in a vacuum. Therefore, it would appear that the molybdenum-copper composite fabricated by the above process would be unacceptable for use as a contact material in vacuum environment due to its high gas content and content of materials which may release gas during the operation of the composite material in a vacuum environment. It is thought that the gas content and the content of materials which may release gas in such a contact material is in excess of 50 parts per million.

It is thought that in order to reduce the gas content of the contact material, infiltration should be carried out in a vacuum atmosphere. A copper melt shows substantially no penetration into a molybdenum powder body in a vacuum using standard metallurgical techniques. It is thought that the lack of penetration of copper into the molybdenum powder body in a vacuum atmosphere may be due to the unfavorable surface energies present in the vacuum atmosphere.

If there is insolubility between the metals as is the case between molybdenum and copper, and if the wetting is poor, an auxiliary agent influencing the surface energies in the desired direction is required in order to achieve infiltration of a powder body of one metal with a melt of a second metal or metal alloy.

In the present invention, by utilizing small amounts of an auxiliary agent or reactive metal selected from the group consisting of titanium and zirconium and by using vacuum infiltration techniques, a melt of metal selected from the group consisting of copper, silver and gold alloyed with a small but significant percent of an auxiliary agent or reactive metal selected from the group consisting of titanium and zirconium infiltrates the voids of the molybdenum powder body so as to provide a substantially voidless composite. It is thought that the agent either raises the surface energies of the melt or of the solid, or lowers the surface energies of the interface between the melt and the solid thereby favoring infiltration of the melt into the molybdenum powder body. It is thought that the vacuum serves the dual functions of assisting penetration of the alloy melt into the molybdenum powder body and of decreasing the content of all gases present. As indicated before, in order for the composite material to be acceptable for operation in a vacuum atmosphere, the composite material should contain a low gas content.

Therefore, it is an object of the present invention to provide a composite material suitable for use as a current carrying material in a vacuum atmosphere.

Another object of the present invention is to provide a means and method of fabricating a composite contact material using vacuum infiltration techniques.

A further object of the present invention is to provide means and methods of fabricating a composite contact material having high electrical and thermal conductivity properties combined with low erosion under arcing and high resistance to welding.

A further object of the present invention is to provide an alloy which includes an auxiliary agent for wetting a molybdenum skeleton, that is ductile, that has high electrical and thermal conductivity, and has a melting point temperature which is lower than that of molybdenum.

A further object of the present invention is to provide a composite material of a substantially continuous skeleton of integrally bonded molybdenum, the voids of which are filled by a substantially continuous matrix of an alloy which is substantially mutually insoluble and substantially nonreactive with the molybdenum for use as an electrical contact material wherein the concentration of a less conductive metal in the alloy matrix has a higher

concentration in the molybdenum interface region than in the region between the molybdenum and the alloy matrix thereby raising the overall conductivity of the alloy matrix.

Another object of the present invention is to provide a means and method of using an alloy which is substantially mutually insoluble and substantially nonreactive with molybdenum as infiltration stock for molybdenum powder bodies so as to allow substantially complete vacuum infiltration of the voids areas of molybdenum powder body thereby providing a composite contact material having a substantially continuous molybdenum skeleton integrally joined with a substantially continuous alloy matrix material.

Another object of the present invention is to provide a current carrying material consisting essentially of a metal alloy which is substantially mutually insoluble and substantially nonreactive with molybdenum, the molybdenum content of the material constituting the majority by volume percent of the material.

A further object of the present invention is to provide a current carrying material consisting of about 55 to 88% by volume molybdenum and about 45 to 12% by volume of an infiltrant which is substantially mutually insoluble and substantially nonreactive with the molybdenum.

The present invention, in another of its aspects, relates to the novel features of the instrumentalities of the invention described herein for teaching the principal object of the invention and to the novel principles employed in the instrumentalities whether or not these features and principles may be used in the said object and/or in the said field.

With the aforementioned objects enumerated, other objects will be apparent to those persons possessing ordinary skill in the art. Other objects will appear in the following description and in the appended claims.

In the drawings:

FIGURE 1 illustrates the several steps involved in the method of making the current carrying material.

FIGURE 2 illustrates the current carrying material.

Generally speaking, the present invention relates to a composite of a substantially continuous skeleton of integrally bonded molybdenum particles, the voids of which are filled by a substantially continuous matrix of an alloy which is substantially mutually insoluble and substantially nonreactive with the molybdenum. The molybdenum content of the composite constitutes the majority by volume percent of the composite.

The method of the present invention relates to contacting a porous sintered or unsintered molybdenum body with an alloy which contains an agent for wetting the molybdenum particles so that the alloy substantially completely infiltrates the body in a vacuum atmosphere.

More particularly, the means and methods of the present invention relate to fabricating a current carrying material consisting essentially of a continuous skeleton of integrally bonded molybdenum particles, the voids of which are filled by a substantially continuous matrix of a metal alloy which is substantially mutually insoluble and substantially nonreactive with molybdenum. The metal metal alloy consists essentially of a first metal selected from the group consisting of copper, gold and silver and a small but significant addition of a second metal selected from the group consisting of titanium and zirconium. Of the first group of metals copper is preferred. Of the second group of metals titanium is preferred.

The molybdenum powder has a particular size ranging from preferably about 1 to 50 microns. The molybdenum particle size may vary in accordance with the desired porosity of the molybdenum powder body. It should be understood that molybdenum powder having a larger or smaller particle size may be used. The powder is compacted in a suitable mold under a pressure sufficient to provide green compacts with sufficient strength to be

handled and with densities which will yield desired composite composition. Compacting pressures ranging from 10 to 30 tons per inch squared resulted in green compacts with desired strength and density. The compact densities

range from about 55-58% of theoretical density. The molybdenum body may be sintered in any suitable non-oxidizing atmosphere such as hydrogen, argon, dissociated ammonia, or vacuum atmosphere for about 1 to 15 hours or more at a temperature of about 1300°-1800° C. The lower the sintering temperature, the longer the sintering time. However, sintering of the compact is not a necessary prerequisite to successful infiltration thereof by the alloy melt. The compact, sintered or unsintered, is placed in a vacuum atmosphere. The vacuum atmosphere may have a pressure of about  $1 \times 10^{-5}$  torrs or harder vacuum. A vacuum pressure of about  $5 \times 10^{-6}$  torrs or harder is preferred. The molybdenum powder body is contacted with the alloy which is substantially mutually insoluble and substantially nonreactive with the molybdenum body.

The molybdenum body, sintered or unsintered, is infiltrated in the vacuum environment with the alloy metal at a temperature sufficiently high to yield a free flowing melt. The infiltration temperature contemplated is about 1100°-1200° C. Attempting infiltration of the body with an alloy composed of the metals contemplated at a temperature below about 1100° C., poor fluidity of the melt is experienced. Attempting infiltration of the body at a temperature in excess of 1200° C., the melt appears to suffer excessive evaporation.

The molybdenum content of the composite material is about 55 to 88% by volume of the total volume of the composite. It is thought that a molybdenum content of less than 55% by volume leads to undesirable contact welding and arc erosion during operation of the contact material. It is thought that a molybdenum content of more than 88% by volume of the total volume of the constituents of the composite material results in an undesirable electrical conductively characteristic of the material. It is thought that the titanium or zirconium alloyed with either copper, gold or silver should not exceed about 0.4% by volume or be less than 0.01% by volume of the total volume of the constituents of the composite. For example, if the reactive metal content of the alloy exceeds about 0.4% by volume, it may result in an alloy matrix having an undesirable conductivity. Using less than about 0.01% by volume may result in seriously impeding the infiltration of the melt into the molybdenum body. The copper, gold or silver content of the total volume of the composite material is about 44.9 to 11.9% by volume.

It is believed that an electron probe analysis of a molybdenum-alloy matrix region will show segregation or high concentration of the titanium or zirconium constituent of the alloy in the interface region between the molybdenum and the alloy metal. Since titanium and zirconium are poorer conductors than either copper, gold or silver, the overall conductivity of the alloy matrix should be raised.

FIGURE 1 shows the several steps in the method used to fabricate the composite illustrated in FIGURE 2.

FIGURE 2 illustrates a molybdenum-copper-titanium composite 10 consisting of the sintered porous skeleton of molybdenum. The voids of the skeleton are filled by a continuous network of an alloy of copper-titanium 12. The copper-titanium alloy is integrally bonded with the molybdenum skeleton.

The following Examples 1 to 3 are illustrative of the preparation of molybdenum-copper-titanium or of a molybdenum-silver-titanium composite contact material fabricated using the vacuum infiltration technique described above.

#### EXAMPLE 1

A molybdenum body vacuum infiltration with an alloy of copper-titanium, the composite consisting essentially of about 72.3% by volume molybdenum, 27.5% by volume copper, the remainder titanium.

Powdered molybdenum having a particle size of about 45 microns or less is pressed by any suitable means such as by an automatic press at a pressure of about 12 tons per square inch to provide a green compact sturdy enough to be handled. The green compact has a compact density of about 73% of theoretical density. The green molybdenum compact is then sintered for about 15 hours at a temperature of about 1300° C. in a hydrogen atmosphere. The sintered compact is contacted with an alloy of copper-titanium in a vacuum atmosphere. The sintered compact and contacting alloy are heated at a temperature of about 1200° C. for about 30 minutes at a pressure of about  $2 \times 10^{-6}$  torrs. The porous molybdenum body is infiltrated with the copper-titanium alloy. The resultant composite is a dense structure having high electrical and thermal conductivity combined with high resistance to deformation under pressure and has a low gas content, that is, a gas content and content of materials which may release gas of no more than 10 p.p.m.

#### EXAMPLE 2

A molybdenum powder body vacuum infiltrated with an alloy of copper-titanium. The composite consists essentially of about 76.5% by volume molybdenum, about 23.3% by volume copper, the remainder titanium.

Molybdenum particles having a particle size of about 45 microns or less is pressed by any suitable means such as by an automatic press at a pressure of about 15 tons per square inch. The compact has a density of about 76% of theoretical density. The green compact is subjected to sintering for 7 hours at a temperature of about 1375° C. The sintered compact has a density of about 76.5% of theoretical density. The sintered compact is contacted with an alloy of copper-titanium in a vacuum atmosphere. The sintered compact and contacting alloy are heated for 30 minutes at a temperature of about 1200° C. at a pressure of about  $2 \times 10^{-6}$  torr. The resultant composite of molybdenum-copper-titanium is a dense structure having high electrical and thermal conductivity characteristics combined with high resistance to deformation under pressure and low gas content, that is, a gas content and content of materials which may release gas of no more than 10 p.p.m.

#### EXAMPLE 3

A molybdenum-silver-titanium composite material may be prepared using the procedure of Example 2. The proportions of the materials of the composite approximate the proportions recited above.

It is thought that the molybdenum powder body or the sintered molybdenum body may be coated with a metal selected from the group of titanium and zirconium by electrolytic or vapor phase plating, impregnation of the coated body could be carried out successfully with essentially pure (unalloyed) copper. Vacuum infiltration should occur as long as either zirconium or titanium is at the boundary. The amount of the plated zirconium or titanium will be such that its composition would amount to about 0.4 to 0.01% by volume of the total volume of the constituents.

The present invention is not intended to be limited to

the disclosure herein, and changes and modifications may be made by those skilled in the art without departing from the spirit and the scope of the present invention. Such modifications and variations are considered to be within the purview and scope of the present invention and the appended claims.

Having thus described our invention, we claim:

1. A current carrying composite material consisting essentially of molybdenum and a metal alloy which is substantially mutually insoluble and substantially non-reactive with the molybdenum, said molybdenum content being the majority percent by volume of the composite, said metal alloy consisting essentially of a metal having a high current conductivity and a metallic wetting agent selected from the group consisting of titanium and zirconium, said agent consisting of up to about 0.4% by volume of the constituents of said current-carrying material.
2. A current carrying material as claimed in claim 1, wherein said high conductivity metal is selected from the group consisting of copper, gold and silver.
3. A current carrying material as claimed in claim 2, wherein said molybdenum is about 55 to 88% by volume and the remainder said alloy.
4. A current carrying material as claimed in claim 3 wherein said high conductivity metal content of said alloy is about 44.9 to 11.9% by volume and said metallic wetting agent content 0.4 to 0.01% by volume.
5. A current carrying material as claimed in claim 4, wherein said molybdenum is a molybdenum skeleton, the voids of which are substantially filled with said alloy, said alloy having a high concentration of said metallic wetting agent in the interface region between said molybdenum and said alloy thereby raising the overall electrical conductivity of said alloy.
6. A current carrying material as claimed in claim 2, wherein said alloy consists of said copper and said titanium.
7. A current carrying material as claimed in claim 6, wherein said molybdenum contents of said material is about 72.3% to about 76.5% by volume, said copper content is about 27.5% to about 23.3% by volume and said titanium content is about 0.2% by volume.
8. A current carrying material as claimed in claim 7, wherein said molybdenum is bonded together molybdenum particles having a particle size of about 1 to about 50 microns, the voids between said particles are substantially filled with said alloy.

#### References Cited

##### UNITED STATES PATENTS

|           |         |           |       |            |
|-----------|---------|-----------|-------|------------|
| 1,848,438 | 3/1932  | Sieger    | ----- | 29—182.1   |
| 2,160,659 | 5/1939  | Hensel    | ----- | 29—182.1   |
| 2,851,381 | 9/1958  | Hoyer     | ----- | 29—182.1 X |
| 3,069,757 | 12/1962 | Beggs     | ----- | 29—182.1   |
| 3,303,559 | 2/1967  | Holtzclaw | ----- | 75—208 X   |
| 3,338,687 | 8/1967  | Dickinson | ----- | 29—182.2 X |

CARL D. QUARFORTH, Primary Examiner.

A. J. STEINER, Assistant Examiner.